# EUROPEAN PATENT SPECIFICATION

(11) **EP 1 414 933 B1**
(45) Date of publication and mention of the grant of the patent: **06.04.2005**
(21) Application number: 02742048.8
(22) Date of filing: 14.06.2002
(51) Int. Cl.: C10L 1/22, C10L 1/14, C10L 10/00

(54) **FUEL COMPOSITION CONTAINING DETERGENT COMBINATION AND METHODS THEREOF**
REINIGUNGSMITTELSZUSAMMENSTELLUNG ENTHALTENDE BRENNSTOFFZUSAMMENSETZUNG UND DEREN VERFAHREN
COMPOSITION DE CARBURANT CONTENANT UNE COMBINAISON DE DETERGENTS ET PROCEDES ASSOCIES

(30) Priority: 07.08.2001 US 924027
(43) Date of publication of application: 06.05.2004
(73) Proprietor: THE LUBRIZOL CORPORATION, Wickliffe, Ohio 44092-2298 (US)
(72) Inventor: JACKSON, Mitchell, M., Chagrin Falls, OH 44022 (US); ARTERS, David, C., Repton, Derbyshire DE65 6FN (GB)
(74) Representative: Mallalieu, Catherine Louise
(86) International application number: PCT/US2002/018749
(87) International publication number: WO 2003/014267

(56) References cited:
- EP-A- 0 534 551
- EP-A- 0 831 141
- US-A- 4 166 726

## Description

### BACKGROUND OF THE INVENTION

### Field of the Invention

This invention involves a fuel composition that includes a combination of detergents and methods that utilize the fuel composition to operate and to control deposits in an internal combustion engine.

### Description of the Related Art

Hydrocarbon fuels generally contain substances that tend to form deposits in the fuel delivery system of an internal combustion engine such as the fuel injectors in diesel engines and the intake valves in gasoline engines. These deposits, if allowed to build up, can significantly reduce engine performance in terms of power output, fuel economy and exhaust emissions. It is highly desirable to incorporate detergents into hydrocarbon fuels that are effective in controlling deposits by inhibiting their formation and facilitating their removal so that engine performance is maintained or improved.

Graiff et al. in European Publication No. EP 534551A1 published on March 31, 1993 disclose a gasoline composition that comprises a gasoline and a mixture of a) a polyamine selected from the group consisting of an aliphatic alkylene polyamine containing at least one olefinic polymer, a Mannich polyamine, and mixtures of the aliphatic alkylene polyamine and the Mannich polyamine and b) a hydrocarbyl poly(oxyalkylene) aminocarbamate.

Cunningham et al. in U.S. Patent No. 5,679,116 issued October 21, 1997 disclose fuel additive compositions comprising a) at least one detergent/dispersant which is a derivative of a hydrocarbon-substituted dicarboxylic acid or anhydride, a hydrocarbon having a polyamine attached, and/or a Mannich condensation product, b) a cyclopentadienyl complex of a transition metal and c) a liquid carrier or additive induction aid.

Croudace et al. in International Publication No. WO 90/10051 published September 7, 1990 disclose a fuel composition comprising a gasoline and an additive combination comprising one or more C₆+ primary amines, one or more gasoline dispersants selected from the group consisting of polyalkylamines and Mannich bases, and a fluidizer oil.

Daly in U.S. Patent No. 5,873,917 issued February 23, 1999 discloses a fuel composition comprising a gasoline, a polyether alcohol, a hydrocarbylphenol, and optionally a third component comprising a nitrogen-containing dispersant to include hydrocarbyl-substituted amines, Mannich dispersants, and polyetheramines.

Wright in U.S. Patent No. 5,169,410 issued December 8, 1992 discloses a method to stabilize gasoline mixtures comprising adding to the gasoline a combination of a phenylenediamine having at least one N-H group and a strongly basic organo-amine comprising a Mannich reaction product.

US-A-4166726 discloses a fuel composition containing a mixture of polyalkylene amine and the reaction product of alkylphenol, aldehyde and amine.

The present invention is directed to a fuel composition that includes a combination of two nitrogen-containing detergents and that is unexpectedly much more effective and efficient in controlling deposits in a hydrocarbon fueled internal combustion engine compared to fuel compositions that include a combination of either nitrogen-containing detergent with a fluidizer.

### SUMMARY OF THE INVENTION

It is an object of the present invention to control deposits in an internal combustion engine so that engine performance is maintained or improved.

An additional object of this invention is to control deposits in a gasoline engine.

Another object of this invention is to control deposits in a diesel engine.

The objects, advantages and embodiments of the present invention are in part described in the specification and in part are obvious from the specification or from the practice of this invention. Therefore, it is understood that the invention is claimed as described or obvious as falls within the scope of the appended claims.

To achieve the foregoing objects in accordance with the invention as described in the wording of independent claim 1, a fuel composition of this invention useful for a spark or a compression ignition internal combustion engine comprises a hydrocarbon fuel, a combination of nitrogen-containing detergents comprising a hydrocarbyl-substituted polyamine and a Mannich reaction product of an alkyl-substituted hydroxyaromatic compound with an aldehyde and a polyamine having at least one reactive N-H group, and optionally a fluidizer comprising a polyether, a polyetheramine, or mixtures thereof where the weight ratio of the hydrocarbyl-substituted polyamine to the Mannich reaction product is about 0.5:1 to 1:0.5, wherein the alkyl substituent of the alkyl-substitued hydroxyaromatic compound is derived from a polyolefin having a number average molecular weight of 900-1500; where each of the nitrogen-containing detergents is present at 20-100 ppm by weight, the combination of nitrogen containing detergents is present at or greater than 60 ppm by weight, and where the weight ratio of the fluidizer to the combination of nitrogen-confining detergents is less than 0.5. Further embodiments of the claimed composition are disclosed in dependent claim 2 to 10.

Another embodiment of this invention is a method of operating an internal combustion engine which comprises fueling the engine with the fuel composition of this invention where the hydrocarbon fuel is a gasoline or a diesel fuel, and where the gasoline or diesel fuel optionally contains an oxygenate comprising methanol, ethanol, methyl tert-butyl ether, ethyl tert-butyl ether, methyl tert-amyl ether, or mixtures thereof.

A further embodiment of this invention is a method of controlling deposits in an internal combustion engine which comprises fueling the engine with the fuel composition of this invention where the hydrocarbon fuel is a gasoline or a diesel fuel, and where the gasoline or diesel fuel optionally contains an oxygenate comprising methanol, ethanol, methyl tert-butyl ether, ethyl tert-butyl ether, methyl tert-amyl ether, or mixtures thereof.

### DETAILED DESCRIPTION OF THE INVENTION

A fuel composition of the present invention useful for a spark or a compression ignition internal combustion engine comprises a hydrocarbon fuel; a combination of nitrogen-containing detergents comprising a hydrocarbyl-substituted polyamine and a Mannich reaction product of an alkyl-substituted hydroxyaromatic compound, an aldehyde and a polyamine having at least one reactive N-H group; and optionally a fluidizer comprising a polyether, a polyetheramine, or mixtures thereof where the weight ratio of the hydrocarbyl-substituted polyamine to the Mannich reaction product is 0.5:1 to 1:0.5, each of the nitrogen-containing detergents is present at 20-100 ppm by weight, and the weight ratio of the fluidizer to the combination of nitrogen-containing detergents is less than 0.5 and the rest of features of independent claim 1.

The hydrocarbon fuel of the present invention is well known to those skilled in the art. Hydrocarbon fuels are generally derived from petroleum by various refinery processes. The hydrocarbon fuel can be a gasoline or a diesel fuel. The gasoline or diesel fuel optionally can contain an oxygenate or oxygen-containing molecule up to a level of 25% by weight of oxygenate. Oxygenates include alcohols, ethers, ketones, esters, nitroalkanes, or mixtures thereof. Commonly used oxygenates include methanol, ethanol, methyl tert-butyl ether, ethyl tert-butyl ether, methyl tert-amyl ether, or mixtures thereof. Gasoline, suitable for use in spark ignition engines, generally boils in the range from 30 to 230°C and has a research octane number typically in the range of 90 to 100. Diesel fuel, suitable for use in compression ignition engines, generally boils in the range from 140 to 400°C and has a cetane number in the range from 25 to 60.

The hydrocarbyl-substituted polyamine of the present invention has a hydrocarbyl substituent with a number average molecular weight of 500 to 5000, preferably 700 to 2000, and more preferably 900 to 1500. The hydrocarbyl substituent is a univalent radical of carbon atoms that is predominantly hydrocarbon in nature but can have nonhydrocarbon substituent groups to include hydroxy groups and can contain heteroatoms. The hydrocarbon substituent can be derived from a polyolefin having a number average molecular weight as described above for the hydrocarbyl substituent. The polyolefin can be a homopolymer derived from one olefin or a copolymer derived from two or more olefins. The olefin can have 2 to 10 carbon atoms and includes ethylene, propylene, butene isomers, decene isomers, and mixtures of two or more thereof. The polyolefin includes polyethylenes, polypropylenes, polybutenes and copolymers of ethylene and propylene. A preferred polyolefin is a polyisobutylene prepared by polymerization of a refinery stream containing 30 to 60% by weight isobutylene using a Lewis acid catalyst such as aluminum trichloride or boron trifluoride. The polyolefin can be a polyisobutylene having at least 70% of its olefin double bonds at a terminal position on the carbon chain as the highly reactive vinylidene isomer which is also described below for the Mannich reaction product.

The polyamine portion of the hydrocarbyl-substituted polyamine of the present invention is derived from a polyamine containing two or more amine nitrogen atoms and having at least one reactive N-H group. The polyamine can be aliphatic, cycloaliphatic, heterocyclic or aromatic and includes alkylenediamines, polyalkylenepolyamines, and hydroxy-containing polyamines. Polyamines that can be used in preparing the hydrocarbyl-substituted polyamine include ethylenediamine, 1,3-propylenediamine, N,N-di-methyl-1,3-propanediamine, N-aminoethylpiperazine, N-aminopropylmorpholine, N,N'-di-butyl-para-phenylenediamine, diethylenetriamine, triethylenetetramine, 2-(2-aminoethylamino)ethanol, and mixtures thereof. In another instance the hydrocarbyl-substituted polyamine is derived from the group consisting of ethylenediamine, diethylenetriamine, N,N-dimethyl-1,3-propanediamine, 2-(2-aminoethylamino)ethanol, and mixtures thereof.

The hydrocarbyl-substituted polyamine can be prepared from the polyolefin and the polyamine as detailed above by several methods as described in U.S. Patent 6,193,767 to include 1) halogenating a polyolefin followed by reaction with a polyamine, 2) hydroformulating a polyolefin followed by reaction with a polyamine and finally hydrogenation of the aldehyde-polyamine reaction intermediate, and 3) epoxidizing a polyolefin followed by reductive amination or amination with a polyamine to form a polyamine or hydroxy-containing polyamine derivative respectively. A preferred method of preparation involves chlorinating a polyisobutylene so that it contains at least one chlorine atom. The chlorinated polyisobutylene is then reacted with the polyamine generally at elevated temperatures of about 120°C or higher. A solvent can be used to facilitate the reaction. Excess polyamine can be used to avoid cross-linking to include dimer formation as well as aid in hydrogen chloride removal although an inorganic base such as sodium hydroxide or sodium carbonate is usually employed to remove the hydrogen chloride. U.S. Patent 5,407,453 describes the method of halogenating a polyolefin followed by reaction with a polyamine.

The Mannich reaction product of the present invention is derived from the reaction of an alkyl-substituted hydroxyaromatic compound, an aldehyde, and a polyamine having at least one reactive N-H group. The hydroxyaromatic portion of the alkyl-substituted hydroxyaromatic compound comprises phenol, ortho-cresol, or mixtures thereof. The alkyl-substituent of the alkyl-substituted hydroxyaromatic compound can be derived from a polyolefin which can be a homopolymer, copolymer, or mixtures thereof. The polyolefin has have a number average molecular weight of 900 to 1500. These polyolefins can be prepared from olefin monomers of 2 to 10 carbon atoms to include ethylene, propylene, isomers of butene, isomers of decene and mixtures of two or more thereof. The polyolefins include polyethylenes, polypropylenes, polybutenes and copolymers of ethylene and propylene. A preferred polyolefin is a polyisobutylene derived from a refinery stream having an isobutylene content of 30 to 60% by weight. A more preferred polyolefin is a polyisobutylene having at least 70% of its olefinic double bonds at a terminal position on the carbon chain as the vinylidene type. Highly reactive polyisobutylenes having a high vinylidene isomer content include Glissopal® marketed by BASF. The alkyl-substituted hydroxyaromatic compound can be prepared by well known methods including alkylating a hydroxyaromatic compound such as phenol with a polyolefin such as polyisobutylene using a Lewis acid catalyst like boron trifluoride.

The aldehyde used to prepare the Mannich reaction product of the present invention can be an aldehyde having 1 to 6 carbon atoms. Formaldehyde is preferred and can be used in one of its reagent forms such as paraformaldehyde and formalin.

The polyamine used to prepare the Mannich reaction product of the present invention contains at least two or more amine nitrogen atoms and has at least one reactive N-H group capable of undergoing the Mannich reaction . The polyamine includes alkylenediamines, polyalkylenepolyamines, polyamines containing hydroxy groups and cyclic polyamines. The Mannich reaction product can be derived from the group consisting of ethylenediamine, propylenediamine, N,N-dimethylethylenediamine, N,N'-dimethylethylenediamine, N,N,N'-trimethylethylenediamine, N,N-dimethylpropylenediamine, N,N'-dimethylpropylenediamine, diethylenetriamine, triethylenetetramine, 2-(2-aminoethylamino)ethanol, 4-(3-aminopropyl)-morpholine, and mixtures thereof.

The Mannich reaction product of the present invention can be prepared by reacting the alkyl-substituted hydroxyaromatic compound, aldehyde and polyamine by well known methods including the method described in U.S. Patent 5,876,468.

The fluidizer of the present invention comprises a polyether, a polyetheramine, or mixtures thereof. The polyether of the present invention can be represented by the formula RO[CH₂CH(R¹)O]ₓH where R is a hydrocarbyl group; R¹ is selected from the group consisting of hydrogen, alkyl groups of 1 to 14 carbon atoms, and mixtures thereof; and x is a number from 2 to 50. The hydrocarbyl group R is a univalent hydrocarbon group as described above for the hydrocarbyl-substituted polyamine, has one or more carbon atoms, and includes alkyl and alkylphenyl groups having 7 to 30 total carbon atoms, preferably 9 to 25 total carbon atoms, and more preferably 11 to 20 total carbon atoms. The repeating oxyalkylene units are preferably derived from ethylene oxide, propylene oxide, and butylene oxide. The number of oxyalkylene units x is preferably 10 to 35, and more preferably 18 to 27. The polyether of the present invention can be prepared by various well known methods including condensing one mole of an alcohol or alkylphenol with two or more moles of an alkylene oxide, mixture of alkylene oxides, or with several alkylene oxides in sequential fashion usually in the presence of a base catalyst. U.S. Patent 5,094,667 provides reaction conditions for preparing a polyether. Suitable polyethers are commercially available from Dow Chemicals, Huntsman, ICI and include the Actaclear® series from Bayer.

The polyetheramine of the present invention can be represented by the formula R[OCH₂CH(R¹)]ₙA where R is a hydrocarbyl group as described above for polyethers; R¹ is selected from the group consisting of hydrogen, alkyl groups of 1 to 14 carbon atoms, and mixtures thereof; n is a number from 2 to 50; and A is selected from the group consisting of ―OCH₂CH₂CH₂NR²R² and ―NR³R³ where each R² is independently hydrogen or a hydrocarbyl group of one or more carbon atoms, and each R³ is independently hydrogen, a hydrocarbyl group of one or more carbon atoms, or ―[R⁴N(R⁵)]ₚR⁶ where R⁴ is C₂-C₁₀ alkylene, R⁵ and R⁶ are independently hydrogen or a hydrocarbyl group of one or more carbon atoms, and p is a number from 1 to 7. The polyetheramine is preferably derived from ethylene oxide, propylene oxide, or butylene oxide. The number of oxyalkylene units n in the polyetheramine is preferably 10 to 35, and more preferably 18 to 27. The polyetheramine of the present invention can be prepared by various well know methods. A polyether derived from an alcohol or alkylphenol as described above can be condensed with ammonia, an amine or a polyamine in a reductive amination to form a polyetheramine as described in European Publication No. EP 310875. Alternatively, the polyether can be condensed with acrylonitrile and the nitrile intermediate hydrogenated to form a polyetheramine as described in U.S. Patent 5,094,667. Polyetheramines where A is ―OCH₂CH₂CH₂NH₂ are preferred. Polyetheramines are commercially available in the Techron® series from Chevron and in the Jeffamine® series from Huntsman.

The fuel composition of the present invention includes a combination of nitrogen-containing detergents comprising a hydrocarbyl-substituted polyamine and a Mannich reaction product as described above which is in a weight ratio of the polyamine to the Mannich reaction product of 0.5:1 to 1:0.5, preferably of 0.75:1 to 1:0.75, and more preferably of 1:1. Each of the nitrogen-containing detergents can be present in the fuel composition at 20-100 ppm by weight, preferably at 22-80 ppm by weight, and more preferably at 24-60 ppm by weight. The fuel composition optionally includes a fluidizer comprising a polyether, a polyetheramine, or mixtures thereof as described above where the weight ratio of the fluidizer to the combination of the nitrogen-containing detergents is less than 0.5, in another embodiment less than 0.3, and in a further embodiment less than 0.2

The fuel composition comprises the combination of nitrogen-containing detergents, the hydrocarbyl-substituted polyamine and Mannich reaction product, at or greater than 60 ppm by weight as illustrated in the examples of Table 1 and 2 hereinbelow.

A method of the present invention of operating an internal combustion engine comprises fueling the engine with the fuel composition of the present invention which comprises the hydrocarbon fuel, the combination of nitrogen-containing detergents, and optionally the fluidizer as described in this application. In another embodiment of the present invention, a method of controlling deposits in an internal combustion engine comprises fueling the engine with the fuel composition of the present invention as described in this application. The benefits of the methods of the present invention are illustrated in the examples of Table 1 and 2 hereinbelow.

The fuel composition of the present invention can include a solvent to facilitate handling and transfer of fuel additives and fuel additive concentrates and to provide homogeneous fuel additive concentrates and fuel compositions. The solvent can be an aliphatic hydrocarbon, aromatic hydrocarbon, glycol ether, alcohol, or mixtures thereof. Examples of suitable solvents include various naphthas, various kerosenes, benzene, toluene, xylenes, aliphatic alcohols having 2 to 10 carbon atoms, or mixtures thereof.

The fuel composition of the present invention can include additional fuel additives depending on the requirements of the engine it is used in. In general the fuel composition can include antioxidants such as hindered phenols, supplemental detergents like succinimides, corrosion inhibitors such as alkenylsuccinic acids, antistatic agents, biocides, demulsifiers, and additional fluidizers such as mineral oils and poly(alpha-olefins). Gasoline fuel compositions can contain antiknock additives such as methylcyclopentadienyl manganese tricarbonyl, haloalkane lead scavengers, and anti-valve seat recession additives such as alkali metal sulphosuccinate salts. Diesel fuel compositions can contain organo nitrite or nitrate cetane improvers, cold flow improvers such as copolymers of ethylene and vinyl acetate, smoke suppressants, antifoam agents like silicone fluids, and lubricity agents such as tall oil fatty acids.

The fuel composition of the present invention is generally prepared by mixing the components which can include the hydrocarbon fuel, the nitrogen-containing detergents, fluidizer, solvent, and additional fuel additives at ambient temperature or at an elevated temperature of 40 to 60°C until the mixture is homogeneous. The various fuel additive and solvent components can be added to the hydrocarbon fuel separately but are usually added as a mixture or fuel additive concentrate which is prepared in the same way as the fuel composition.

The patent documents cited in this application regarding methods of preparation are incorporated herein by reference for their disclosure of these methods of preparation.

The advantages of the present invention in controlling deposits in an internal combustion engine are illustrated in the following examples in Table 1 and 2.

**Table 1**

| BMW^{a} 2,500 Miles with Unleaded Gasoline Containing Ethanol | | | | | |
|---|---|---|---|---|---|
| Example | A Hydrocarbyl Polyamine^{b}, ppm actives | B Mannich^{c}, ppm actives | Fluidizer, Ppm actives | Ratio of Fluidizer to A + B | Intake Valve Deposits, mg |
| 1 (comparative) | 61.6 | ― | 31.6^{d} | 0.51 | 282 |
| 2 (comparative) | 68.4 | ― | 35.1^{d} | 0.51 | 85 |
| 3 (comparative) | 30.2 | ― | 46.4^{e} | 1.54 | 172 |
| 4 | 31.7 | 32.7 | 3.9^{c} | 0.06 | 48 |
| 5 | 36.0 | 37.1 | ― | ― | 43 |

| | | | | | |
|---|---|---|---|---|---|
| ^{a}Fuel induction system deposit test run in BMW vehicle on intake valve deposits for 2,500 miles test cycle. | | | | | |
| ^{b}Hydrocarbyl-substituted polyamine from condensation of chlorinated 1300 molecular weight polyisobutylene and ethylenediamine. | | | | | |
| ^{c}Mannich reaction product of a) alkylphenol from 1000 molecular weight high vinylidene polyisobutylene, b) formaldehyde and c) ethylenediamine. | | | | | |
| ^{d}Polyether from one mole of C₁₂₋₁₅ linear alcohol condensed with 22-24 moles of propylene oxide. | | | | | |
| ^{e}Polyetheramine from one mole of C₁₂₋₁₅ linear alcohol condensed with 22-24 moles of propylene oxide, then cyanoethylation of the propoxylated alcohol with acrylonitrile and hydrogenation of the nitrile intermediate to form the polyetheramine. | | | | | |

**Table 2**

| BMW^{a} 2,500 Miles with Unleaded Gasoline | | | | | |
|---|---|---|---|---|---|
| Example | A Hydrocarbyl Polyamine^{b}, ppm actives | B Mannich^{c}, ppm actives | Polyether^{d}, ppm actives | Ratio of Polyether to A + B | Intake Valve Deposits, mg |
| 6 (comparative) | 68.4 | ― | 35.1 | 0.51 | 25.4 |
| 7 (comparative) | ― | 57.5 | 28.3 | 0.49 | 23.0 |
| 8 | 40.0 | 41.2 | ― | ― | 8.6 |

| | | | | | |
|---|---|---|---|---|---|
| ^{a}Fuel induction system deposit test run in BMW vehicle on intake valve deposits for 2,500 miles test cycle. | | | | | |
| ^{b}Hydrocarbyl-substituted polyamine from condensation of chlorinated 1300 molecular weight polyisobutylene and ethylenediamine. | | | | | |
| ^{c}Mannich reaction product of a) alkylphenol from 1000 molecular weight high vinylidene polyisobutylene, b) formaldehyde and c) ethylenediamine. | | | | | |
| ^{d}Polyether from one mole of C₁₂₋₁₅ linear alcohol condensed with 22-24 moles of propylene oxide. | | | | | |

## Claims

1. A fuel composition useful for a spark or a compression ignition internal combustion engine, comprising:
a hydrocarbon fuel;
a combination of nitrogen-containing detergents comprising a hydrocarbyl-substituted polyamine and a Mannich reaction product of an alkyl-substituted hydroxyaromatic compound, an aldehyde, and a polyamine having at least one reactive N-H group; and
optionally a fluidizer comprising a polyether, a polyetheramine, or mixtures thereof;
wherein the alkyl substituent of the alkyl-substituted hydroxyaromatic compound is derived from a polyolefin having a number average molecular weight of 900-1500; the weight ratio of the hydrocarbyl-substituted polyamine to the Mannich reaction product is 0.5:1 to 1:0.5; each of the nitrogen-containing detergents is present at 20-100 ppm by weight; the combination of nitrogen-containing detergents is present at or greater than 60 ppm by weight; and the weight ratio of the fluidizer to the combination of nitrogen-containing detergents is less than 0.5.

2. The fuel composition of claim 1 wherein each of the nitrogen-containing detergents is present at 22-80 ppm by weight.

3. The fuel composition of claim 1 wherein the weight ratio of the fluidizer to the combination of nitrogen-containing detergents is less than 0.3.

4. The fuel composition of claim 1 wherein the hydrocarbyl substituent of the hydrocarbyl-substituted polyamine is derived from a polyolefin having a number average molecular weight of 900-1500.

5. The fuel composition of claim 4 wherein the polyolefin is a polyisobutylene.

6. The composition of claim 4 wherein the hydrocarbyl-substituted polyamine is derived from the group consisting of ethylenediamine, diethylenetriamine, N,N-dimethyl-1,3-propanediamine, 2-(2-aminoethylamino)ethanol, and mixtures thereof.

7. The fuel composition of claim 1 wherein the hydroxyaromatic portion of said alkyl-substituted hydroxyaromatic compound comprises phenol, ortho-cresol, or mixtures thereof.

8. The fuel composition of claim 7 wherein the polyolefin is a polyisobutylene having at least 70% of the olefinic double bonds as vinylidene double bonds.

9. The fuel composition of claim 8 wherein the aldehyde is formaldehyde; and the Mannich reaction product is derived from the group consisting of ethylenediamine, propylenediamine, diethylenetriamine, N,N'-dimethylethylenediamine, N,N,N'-trimethylethylenediamine, N,N-dimethylethylenediamine, N,N-dimethylpropylenediamine, N,N'-dimethylpropylenediamine, 2-(2-aminoethylamino)ethanol, and mixtures thereof.

10. The fuel composition of any preceding claim wherein the hydrocarbon fuel is a gasoline or a diesel fuel; and wherein the gasoline or diesel fuel optionally contains an oxygenate comprising methanol, ethanol, methyl tert-butyl ether, ethyl tert-butyl ether, methyl tert-amyl ether, or mixtures thereof.

11. A method of operating an internal combustion engine, comprising fueling the engine with the fuel composition of claim 10.

12. A method of controlling deposits in an internal combustion engine, comprising fueling the engine with the fuel composition of claim 10.

## Patentansprüche

1. Brennstoffzusammensetzung, die für einen Verbrennungsmotor mit einer Funken- oder einer Kompressionszündung geeignet ist, umfassend:
einen Kohlenwasserstoffbrennstoff,
eine Kombination von stickstoffhaltigen Detergenzien, die ein Hydrocarbyl-substituiertes Polyamin und ein Mannich-Reaktionsprodukt einer Alkyl-substituierten hydroxyaromatischen Verbindung, eines Aldehyds und eines Polyamins mit mindestens einer reaktiven N-H-Gruppe umfasst, und
gegebenenfalls einen Verflüssiger, der einen Polyether, ein Polyetheramin oder Gemische davon umfasst,
wobei der Alkylsubstituent der Alkyl-substituierten hydroxyaromatischen Verbindung von einem Polyolefin mit einem Molekulargewicht-Zahlenmittel von 900 bis 1 500 abstammt, das Gewichtsverhältnis des Hydrocarbyl-substituierten Polyamins zu dem Mannich-Reaktionsprodukt 0,5:1 bis 1:0,5 beträgt, jedes der stickstoffhaltigen Detergenzien bei 20 bis 100 ppm nach Gewicht vorhanden ist, die Kombination von stickstoffhaltigen Detergenzien bei oder größer als 60 ppm nach Gewicht vorhanden ist und das Gewichtsverhältnis des Verflüssigers zu der Kombination von stickstoffhaltigen Detergenzien weniger als 0,5 beträgt.

2. Brennstoffzusammensetzung nach Anspruch 1, wobei jedes der stickstoffhaltigen Detergenzien bei 22 bis 80 ppm nach Gewicht vorhanden ist.

3. Brennstoffzusammensetzung nach Anspruch 1, wobei das Gewichtsverhältnis des Verflüssigers zu der Kombination von stickstoffhaltigen Detergenzien weniger als 0,3 beträgt.

4. Brennstoffzusammensetzung nach Anspruch 1, wobei der Hydrocarbylsubstituent des Hydrocarbyl-substituierten Polyamins von einem Polyolefin mit einem Molekulargewicht-Zahlenmittel von 900 bis 1 500 abstammt.

5. Brennstoffzusammensetzung nach Anspruch 4, wobei das Polyolefin ein Polyisobutylen ist.

6. Zusammensetzung nach Anspruch 4, wobei das Hydrocarbyl-substituierte Polyamin von der Gruppe abstammt, die aus Ethylendiamin, Diethylentriamin, N,N-Dimethyl-1,3-propandiamin, 2-(2-Aminoethylamino)ethanol und Gemischen davon besteht.

7. Brennstoffzusammensetzung nach Anspruch 1, wobei der hydroxyaromatische Teil der Alkyl-substituierten hydroxyaromatischen Verbindung Phenol, ortho-Cresol oder Gemische davon umfasst.

8. Brennstoffzusammensetzung nach Anspruch 7, wobei das Polyolefin ein Polyisobutylen ist, wobei mindestens 70% der olefinischen Doppelbindungen als Vinylidendoppelbindungen vorliegen.

9. Brennstoffzusammensetzung nach Anspruch 8, wobei der Aldehyd Formaldehyd ist und das Mannich-Reaktionsprodukt von der Gruppe abstammt, die aus Ethylendiamin, Propylendiamin, Diethylentriamin, N,N'-Dimethylethylendiamin, N,N,N'-Trimethylethylendiamin, N,N-Dimethylethylendiamin, N,N-Dimethylpropylendiamin, N,N'-Dimethylpropylendiamin, 2-(2-Aminoethylamino)-ethanol und Gemischen davon besteht.

10. Brennstoffzusammensetzung nach einem der vorstehenden Ansprüche, wobei der Kohlenwasserstoffbrennstoff ein Benzin- oder ein Dieselbrennstoff ist und wobei der Benzin- oder Dieselbrennstoff gegebenenfalls eine sauerstofftragende Komponente enthält, die Methanol, Ethanol, Methyl-tert-butylether, Ethyltert-butylether, Methyl-tert-amylether oder Gemische davon umfasst.

11. Verfahren zum Betreiben eines Verbrennungsmotors, das ein Versorgen des. Motors mit der Brennstoffzusammensetzung nach Anspruch 10 umfasst.

12. Verfahren zum Steuern von Ablagerungen in einem Verbrennungsmotor, das ein Versorgen des Motors mit der Brennstoffzusammensetzung nach Anspruch 10 umfasst.

## Revendications

1. Composition de carburant utile pour un moteur à combustion interne à allumage par étincelle ou par compression, comprenant :
un hydrocarbure ;
une combinaison de détergents contenant de l'azote comprenant une polyamine hydrocarbyl-substituée et un produit de réaction de Mannich d'un composé hydroxyaromatique alkyl-substitué, d'un aldéhyde et d'une polyamine ayant au moins un groupe N-H réactif ; et
éventuellement un fluidifiant comprenant un polyéther, une polyétheramine, ou des mélanges de ceux-ci ;
dans laquelle le substituant alkyle du composé hydroxyaromatique alkyl-substitué est dérivé d'une polyoléfine ayant une masse moléculaire moyenne en nombre de 900 à 1500 ; le rapport pondéral de la polyamine hydrocarbyl-substituée au produit de réaction de Mannich est de 0,5:1 à 1:0,5 ; chacun des détergents contenant de l'azote est présent à raison de 20 à 100 ppm en poids ; la combinaison de détergents contenant de l'azote est présente à raison d'au moins 60 ppm en poids ; et le rapport pondéral du fluidifiant à la combinaison de détergents contenant de l'azote est inférieur à 0,5.

2. Composition de carburant selon la revendication 1, dans laquelle chacun des détergents contenant de l'azote est présent à raison de 22 à 80 ppm en poids.

3. Composition de carburant selon la revendication 1, dans laquelle le rapport pondéral du fluidifiant à la combinaison de détergents contenant de l'azote est inférieur à 0,3.

4. Composition de carburant selon la revendication 1, dans laquelle le substituant hydrocarbyle de la polyamine hydrocarbyl-substituée est dérivé d'une polyoléfine ayant une masse moléculaire moyenne en nombre de 900 à 1500.

5. Composition de carburant selon la revendication 4, dans laquelle la polyoléfine est un polyisobutylène.

6. Composition selon la revendication 4, dans laquelle la polyamine hydrocarbyl-substituée est dérivée du groupe constitué de l'éthylènediamine, de la diéthylènetriamine, de la N,N-diméthyl-1,3-propanediamine, du 2-(2-aminoéthylamino)éthanol, et de mélanges de ceux-ci.

7. Composition de carburant selon la revendication 1, dans laquelle la fraction hydroxyaromatique dudit composé hydroxyaromatique alkyl-substitué comprend du phénol, de l'ortho-crésol ou des mélanges de ceux-ci.

8. Composition de carburant selon la revendication 7, dans laquelle la polyoléfine est un polyisobutylène ayant au moins 70 % des doubles liaisons oléfiniques sous forme de doubles liaisons vinylidène.

9. Composition de carburant selon la revendication 8, dans laquelle l'aldéhyde est le formaldéhyde ; et le produit de réaction de Mannich est dérivé du groupe constitué de l'éthylènediamine, de la propylènediamine, de la diéthylènetriamine, de la N,N'-diméthyléthylènediamine, de la N,N,N'-triméthyléthylènediamine, de la N,N-diméthyléthylènediamine, de la N,N-diméthylpropylènediamine, de la N,N'-diméthylpropylènediamine, du 2-(2-aminoéthylamino)éthanol, et des mélanges de ceux-ci.

10. Composition de carburant selon l'une quelconque des revendications précédentes, dans laquelle l'hydrocarbure est un carburant essence ou diesel ; et dans laquelle le carburant essence ou diesel contient éventuellement un oxygénat comprenant le méthanol, l'éthanol, le méthyl-tert-butyléther, l'éthyl-tert-butyléther, le méthyl-tert-amyléther, ou des mélanges de ceux-ci.

11. Procédé d'actionnement d'un moteur à combustion interne, comprenant l'alimentation du moteur en la composition de carburant selon la revendication 10.

12. Procédé de contrôle des dépôts dans un moteur à combustion interne, comprenant l'alimentation du moteur en la composition de carburant selon la revendication 10.
